

# UNITED STATES PATENT OFFICE.

LUDWIG SCHERBEL, OF BUSSI, AQUILA, ITALY, ASSIGNOR TO SOCIETA ITALIANA DI ELETTROCHIMICA, OF ROME, ITALY.

## PROCESS FOR MANUFACTURING IRON-OXID CASTINGS.

1,163,467.

Specification of Letters Patent.

Patented Dec. 7, 1915.

No Drawing.

Application filed August 1, 1914. Serial No. 854,570.

To all whom it may concern:

Be it known that I, LUDWIG SCHERBEL, a subject of the Emperor of Germany, and residing at Bussi, Province of Aquila, Italy, have invented certain new and useful Improvements in Processes for Manufacturing Iron-Oxid Castings, of which the following is a specification.

The invention relates to an improved process for manufacturing iron oxid castings, and has for its object to obtain castings which are rich in ferric oxid by using the almost worthless burnt pyrites or other iron oxids, without special regard to purity, or metallic iron itself.

Many methods have been devised for making iron oxid castings depending on the fusion in the electric furnace of iron oxids or the oxidation of metallic iron, with a view to casting articles adapted to resist chemical actions and having a small degree of fragility; they are composed of magnetite or similar bodies.

It is known that when iron oxid is melted, a dissociation of the ferric oxid into ferrous oxid



occurs near the melting point, so that mixtures are obtained in which the ratio

$$\frac{\% \text{Fe}_2\text{O}_3}{\% \text{FeO}}$$

is less than 2.21 that is to say, less than this ratio in magnetite,  $\text{FeO} \cdot \text{Fe}_2\text{O}_3$ . These mixtures are fragile and not very resistant to chemical and mechanical action, being mixtures of  $\text{FeO}$  and  $\text{Fe}_2\text{O}_4$ , as may be proved by micrographic analysis. To avoid this

inconvenience, the various methods hitherto devised are directed to converting mixtures rich in  $\text{FeO}$  into magnetite or similar compounds, especially of the form  $\text{FeO} \cdot \text{Fe}_2\text{O}_3$ , by adding ferric oxid, as described in the

German patent Griesheim 193367, or by adding other oxids, especially oxids isomorphous with  $\text{Fe}_2\text{O}_3$ , or by treating the melted oxids with gases containing oxygen, for instance, air, as described in the Italian Patents Nos. 75119 and 75135, granted to the Società Italiana di Elettrochimica. Other methods comprise processes for obtaining magnetite by burning iron in oxygen or

some other oxidizing agent. By these processes, magnetite is obtained which yields 55 castings of higher chemical and mechanical resistance and more easily yielding sound castings. All the known methods however are not easily carried out and they require the use of raw material of high purity, besides careful and costly supervision, while giving, at the best hypothesis, castings having the composition of the magnetic iron oxid which are not sufficiently resistant to 60 chemical agents.

By my invention, castings are obtained which possess a much higher resistance to 65 chemical and mechanical action, and are more easily cast sound, even when using impure raw materials with even 10-15% and 70 upward of foreign substances. For this purpose, instead of stopping at magnetite in which the ratio

$$\frac{\% \text{Fe}_2\text{O}_3}{\% \text{FeO}}$$

75

is equal to 2.21, oxid mixtures are obtained in which this ratio is higher than 3 until they come near to ferric oxid  $\text{Fe}_2\text{O}_3$ . I attain this ratio of three and exceed it at will, 80 by oxidizing under pressure the mass of melted oxids with oxygen or gases rich in oxygen (also air), previously heated or not, or by treating the mass with oxygen-carrying agents, and further by strongly stirring 85 the melted mass. The operation must be carried out quickly, so as to prevent the solidification of the mass which becomes pasty toward  $1350^\circ \text{C}$ , and while operating with a large excess of gas so as to have an 90 excess of pressure such as will prevent the dissociation



The castings must further be cast while 95 injecting oxidizing gas in order to avoid the dissociation also during pouring.

My method is carried out by injecting the oxidizing gas into the mass directly melted in the closed electric furnace, or by 100 pouring the mass from the furnace into a species of converter, or other suitable means, where the oxidizing gas is injected, or by treating the melted oxids with oxygen-carrying agents so that an excess of oxygen 105 is developed. The castings thus obtained

are composed nearly exclusively of  $Fe_2O_3$ , and they have not, like the castings of magnetite, a structure with large crystalline grains, but a compact, homogeneous and 5 very fine structure without blisters which produce holes in the cast articles. This structure which is apparent already with a ratio of the oxids equal to 3, comes out more distinctly when approaching the composition of  $Fe_2O_3$ . These castings are adapted for the most varied uses on account of their good chemical and mechanical qualities.

The process may be used for the oxidation 15 not only of iron oxids and of metallic iron, but also of mixtures of different oxids as set forth in the Italian Patent No. 75135, such as mixtures of iron oxids with oxids of manganese, tungsten, titanium, chromium, 20 vanadium, cobalt, nickel, molybdenum, uranium or the like.

What I claim is:

1. The herein described process for man-

ufacturing iron oxid castings composed of mixtures in which the ratio

$$\frac{\% Fe_2O_3}{\% FeO}$$

is more than 3 and which may attain the 30 composition  $Fe_2O_3$ , by treating a melted iron containing bath with oxygen under pressure and while intimately stirring the mass and then casting the produced oxids in an oxidizing atmosphere.

2. The process of manufacturing iron 35 oxids which consists in treating impure iron oxid with oxygen under pressure and while stirring, and thereafter casting the produced oxids in suitable molds.

In testimony whereof I have signed my 40 name in the presence of two subscribing witnesses the 16th day of July 1914.

DR. LUDWIG SCHERBEL.

Witnesses:

GIOVANNI VALATELLI,  
CORELLO FONTANI.